

## UNITED STATES PATENT OFFICE.

JAMES EDWARD SOUTHCOLBE, OF BIRKENHEAD, AND HENRY MATTHEW WELLS, OF LONDON, ENGLAND.

## LUBRICATING OIL AND THE MANUFACTURE THEREOF.

No Drawing.

Application filed May 28, 1921. Serial No. 473,308.

(GRANTED UNDER THE PROVISIONS OF THE ACT OF MARCH 3, 1921, 41 STAT. L., 1313.)

*To all whom it may concern:*

Be it known that we, JAMES EDWARD SOUTHCOLBE and HENRY MATTHEW WELLS, subjects of the King of Great Britain, residing at Birkenhead, in the county of Chester, England, and London, England, respectively, have invented certain new and useful Improvements in and Relating to Lubricating Oils and the Manufacture Thereof (for which we have filed the following application in England, Feb. 27, 1920, No. 5913), of which the following is a specification.

This invention relates to lubricating oils and to methods of manufacturing and refining the same.

In our United States Patent No. 1,319,129 we describe the manufacture of lubricating oils containing small quantities of substances which lower the surface tension of said oil against water, and in particular describe lubricating oils containing minute quantities of free organic acid.

According to the present invention we conduct the refining of crude hydrocarbon oil in such manner that undesirable impurities are eliminated but that predetermined or adequate quantities of free organic acids either natural or formed during the usual refining processes, are deliberately retained in the oil. Such selectively refined oils are then highly satisfactory lubricants owing to their content of free organic acid in limited amount, although such products may subsequently be blended with other oils, either containing free acid or not, in order to increase or decrease their free acidity. The final content of free acid in the finished lubricating oil should be less than two per cent.

The invention is primarily concerned with the refining of oils which are usually treated by sulphuric acid followed by washing with caustic soda, or to similar processes, e. g. processes of treatment with liquid sulphur dioxide or processes in which the material is subsequently distilled or otherwise treated with alkaline materials such as lime.

For example, Texas crude oil contains large quantities of sulphur or impurities

containing sulphur, or asphaltic impurities and of organic acids or the like. We may interpolate that in this specification we use the term "acid" to include the allied bodies naturally occurring in the oil or formed therefrom during the refining process such as phenolic bodies. In a preferred form of our invention we treat the crude oil with sulphuric acid or the like in order to eliminate the asphaltic impurities and we remove in known manner the sulphur impurities when such are present, but instead of treating with alkaline material so as to remove the whole or practically the whole of the organic acids present, or the organic acids (sulphonic acid in particular) formed by the action of the sulphuric acid or other chemical refining agent, we wash the chemically refined oil with water to such an extent as to remove the free mineral acid, whereupon a lubricating oil is obtained which contains no free mineral acid, but contains limited quantities of free organic acid which improves the lubricating power.

## Example.

A Texas crude oil is refined with sulphuric acid in known manner. The refined oil is then washed with water (instead of with alkali) in several stages. The wash water is repeatedly tested until it is ascertained that the whole of the sulphuric acid has been removed. The washing is then discontinued at a stage when the oil still contains a material quantity of free organic acid, and this amount may be controlled by the amount of washing. If washing is continued until the acid is  $\frac{1}{2}\%$  (calculated as oleic), the oil is then suitable for use as a lubricant.

We declare that what we claim is:

1. The process of manufacturing lubricating oils which consists in refining crude hydrocarbon oils by acid treatment to remove undesirable impurities but to leave after washing out mineral acid a finished oil containing a material amount of organic acid, namely less than two per cent, but enough to reduce the frictional coefficient of said oil by a substantial amount.

2. The process of manufacturing lubricat-

ing oils which consists in refining crude hydrocarbon oils by acid treatment to remove undesirable impurities but to leave in small quantities of organic acids, and then blending said oil with other oil to reduce the free acidity so that the final product contains less than two per cent of organic acid.

In witness whereof we have hereunto signed our names this 11th and 13th days of

May, 1921, in the presence of two subscribing witnesses.

JAMES EDWARD SOUTHCOMBE.  
HENRY MATTHEW WELLS.

Witnesses as to signature of James Edward Southcombe.

H. J. GREGORY,  
JAMES C. MCRAE.